

A. G. JONES.

METALLIZING PROCESS AND APPARATUS.

APPLICATION FILED MAR. 26, 1914. RENEWED JAN. 20, 1916.

1,174,730.

Patented Mar. 7, 1916.

2 SHEETS—SHEET 1.



Witnesses:

C. G. Floyd

Sam. C. Donnan

Inventor:

Albert G. Jones  
Baldwin, Pa., Crittenden, Ky.  
Atty's

A. G. JONES.

METALLIZING PROCESS AND APPARATUS.

APPLICATION FILED MAR. 26, 1914, RENEWED JAN. 20, 1916.

1,174,730.

Patented Mar. 7, 1916.

2 SHEETS—SHEET 2.

Fig. 2.



Witnesses:

John Saylor.

Irvin C. Bournam.

Inventor:

Albert G. Jones,

By his attorney Clinton C. Miller,

Attest:

# UNITED STATES PATENT OFFICE.

ALBERT G. JONES, OF IRON MOUNTAIN, MICHIGAN, ASSIGNEE TO NEW METALS-  
PROCESS COMPANY, OF CHICAGO, ILLINOIS, A CORPORATION OF ILLINOIS.

## METALLIZING PROCESS AND APPARATUS.

1,174,730.

Specification of Letters Patent. Patented Mar. 7, 1916.

Application filed March 26, 1914, Serial No. 827,359. Renewed January 20, 1916. Serial No. 78,179.

To all whom it may concern:

Be it known that I, ALBERT G. JONES, a citizen of the United States, residing at Iron Mountain, in the county of Dickinson 5 and State of Michigan, have invented a new and useful Metallizing Process and Apparatus, of which the following is a specification.

The present invention relates to a process 10 for metallizing ores containing metals which volatilize at a low temperature, notably zinc and lead, which volatilize at a temperature of approximately 2200° F.

The primary object is to provide a thoroughly practicable direct process and apparatus for metallizing zinc and lead oxides and carbonates. The purpose is to de-oxidize the ores and recover the metals, without 15 effecting any general fusing of the earthy constituents, or gangue, or producing a bath of the earthy constituents. Inasmuch as zinc and lead volatilize at a temperature not much above the de-oxidizing temperature, special care is necessary to secure 20 the desired results, and it is desirable to make special provision to prevent re-oxidation of the metals.

According to the preferred method of 25 practising the process herein described, the ore, preferably crushed to 1 inch dimensions or smaller, is mixed with several times its volume of coke, or charcoal, together with a relatively small amount of fuel containing hydrocarbons, such as bituminous 30 coal or wood; and the charge is introduced 35 into a de-oxidizing-chamber where the ore-lump groups, or ore-portions, are maintained practically isolated and surrounded by the fuel; and a temperature is provided 40 which is sufficient to metallize the ore, fuse the same and vaporize a large portion thereof, but without producing a bath of the earthy constituents. The de-oxidizing-gas 45 and metal vapors are then drawn through a condenser where the metals are condensed and recovered in a fluid state, the conditions being such as to prevent re-oxidation of the metals. The unconsumed solid coke (or 50 charcoal) and the gangue in solid form are removed by means of a discharging-device at the bottom of the de-oxidizing-chamber, and the coke is separated and fed again through the furnace with a fresh charge of ore and a sufficient amount of fresh fuel to 55 maintain the proportions. Any metals which

may pass through the de-oxidizing-chamber without vaporizing, or which may cool to a liquid in the de-oxidizing chamber, will coalesce in pools or globules, and may run together and be recovered at the bottom of 60 the de-oxidizing-chamber.

The accompanying drawings illustrate apparatus adapted to the practice of the improved process.

In the drawings—Figure 1 represents an 85 elevational view, partly in section, of the preferred apparatus for practising the process; and Fig. 2 represents an enlarged vertical sectional view of the de-oxidizing-chamber employed.

In the construction illustrated, A represents a de-oxidizing-chamber; B, a condenser; C, a pump; and D, a gasometer.

The de-oxidizing-chamber A preferably is of circular form and provided with a 75 base-portion 1 surmounted by a dome 2. At the junction of the base-portion and dome-portion is a bustle-pipe or annular flue 3 with which the interior of the chamber communicates through passages 3<sup>a</sup>. A 80 flue 3<sup>b</sup> leads from the bustle-pipe 3 to the condenser B.

The base-portion 1 is provided with the interior downwardly-convergent frusto-conical surface 1<sup>a</sup> at the lower end of which is provided a discharge-device 4, which is shown in the form of a slide, which may be hydraulically actuated. The slide 4 is provided with chambers or passages 4<sup>a</sup> and 4<sup>b</sup> which are adapted to discharge the solid 85 materials through lateral openings 5 in the base-portion 1. A shallow collecting-chamber 6 below the slide 4 may serve to collect any fluid metals and discharge the same 90 through a pipe 6<sup>a</sup> to a tank or container 6<sup>b</sup>. 95

The upper end of the chamber A is provided with a hopper 7 fitted with a slide or closure 8. Below the closure 8 is a twyer or twyers 9 provided with air-regulating means 9<sup>a</sup>. Water-coils 10 may be used at 100 the neck-portion of the de-oxidizing-chamber for cooling purposes.

The condenser B may comprise an inclined water-cooled chamber, as shown. A draw-off pipe 11 connects the lower end of 105 the condenser B with the tank 12. A flue 13 leads from the upper portion of the condenser to the pump, from which a pipe 14 leads to the gasometer D.

In the practice of the process, charges of 110

ore and fuel are from time to time introduced through the hopper 7, the closure 8 being withdrawn to permit this operation, and then closed. The fuel is preferably 5 mainly in the form of large lumps or blocks adapted to space or isolate the ore-portions and envelop them with solid carbonaceous fuel. The fuel is preferably several times as heavy as the ore and of many times the 10 volume of the ore. For illustration, the ore and fuel may be fixed in the proportions of 250 pounds of ore, 400 pounds of coke, and 100 pounds of bituminous coal, the volume of the fuel thus being many times the 15 volume of the ore. The chamber A is kept practically full, fresh charges of ore and fuel being introduced from time to time. In Fig. 2, the dotted lines 15 may indicate the upper conical surface of the ore and 20 fuel body. The operation is carried on under conditions to produce a hot zone at the upper portion of the ore body, sufficient air being supplied through the twyvers 9 to effect this result. Carbon dioxid is formed 25 in the upper zone, and this changes to a de-oxidizing gas a short distance below the upper end of the chamber. A temperature ranging upwardly above 2000° F. is desirable in the upper portion of the de-oxidizing-chamber, and the temperature falls as 30 the lower portion of the de-oxidizing-chamber is approached. The de-oxidizing gases are drawn through the flue 3<sup>b</sup> and pass through the condenser B, where the zinc and lead are condensed to form a bath 35 which runs into the collecting-tank 12. The gaseous fuel then passes through the pump C to the gasometer, where it is available for any desired use.

40 It is desirable to employ a de-oxidizing-chamber which will cause the mixture of fuel and ore to assume the condition of a relatively-low stack so that the gases may be drawn readily through the mixture without the expenditure of great power. If desired, the gases may pass from the condenser B through a relatively high stack 16, as indicated by dotted lines in Fig. 1, the stack 16 then taking the place of the pump and gasometer. In such case, the operation 45 may be carried on by natural-draft, owing to the fact that but little pressure is required to force the gases through the low stack of fuel and ore above the outlets 3<sup>a</sup>.

50 The unused coke and the gangue in solid form settle down through the converging lower portion of the chamber A, and the device 4 is operated from time to time to discharge portions of the gangue and coke through the openings 5. Any metals which may be cooled or condensed in the lower portion of the chamber A will collect in small pools or globules on the solid fuel and may run together in the depression 6 and 55 pass to the collecting-tank 6<sup>b</sup>. Any metals

which may become "frozen" will be discharged with the coke and gangue through the openings 5. The coke may be separated and used again, so that any metal globules which may adhere will, in the next passage 70 through the chamber A, be fused and vaporized, or fused and coalesced with other metal particles and collected at the bottom of the de-oxidizing-chamber.

In place of coke and coal, charcoal and 75 wood may be employed as fuel, in which case the volume of fuel, as compared with the volume of ore, will be disproportionately greater. The wood may be 16 inch cord-wood, or slab-wood, and fresh charcoal will be continuously formed in the 80 operation to replenish the charcoal which is consumed.

It may be noted that the relatively small 85 amount of coal or wood which is employed from time to time to replenish the coke or charcoal furnishes hydrocarbons which aid in the reducing action. The temperature should not be so high as to effect any general fusing of the slag constituents of the 90 ore, and the use of so large an excess of solid fuel aids in preventing the formation of a bath as well as serving to envelop or isolate the ore-portions which are undergoing reduction.

95 A furnace having a diameter at the bustle-line of 20 feet preferably has a height above the bustle-line of approximately 10 feet. The air-twyvers 9 may be of a diameter of 20 inches, in which case six or eight twyvers should furnish ample air.

In some cases, it may be desirable to employ blocks of resistant material, such as silica-boulders, together with sufficient fuel to effect the de-oxidizing and vaporizing action. In such case, the refractory stones would serve as spacers, and if coke or charcoal were used in connection therewith, this fuel would also afford spacers.

105 It is to be noted that whether the zinc, for instance, is volatilized as an oxid or as a metal—a question about which there has been difference of opinion—the desired result can nevertheless be attained, since there will in any case be a metal vapor which can 110 be condensed.

The foregoing detailed description has been given for clearness of understanding only, and no unnecessary limitation should be understood therefrom, but the appended 115 claims should be construed as broadly as permissible in view of the prior art.

What I regard as new and desire to secure by Letters Patent is—

1. The process of recovering from ores 125 metals having a comparatively low volatilizing point, which consists in subjecting, in a de-oxidizing chamber, a slowly-settling charge of ore mixed with lump fuel of several times its volume sufficient to maintain 130

- the ore-groups in substantial isolation to a limited down-draft air-supply and producing a temperature sufficient to effect de-oxidation and vaporization, without producing
- 5 a bath of the gangue, maintaining the de-oxidizing conditions, passing the de-oxidizing gas and metal vapor through a condenser in which the de-oxidizing conditions are maintained and the values recovered in
- 10 metallic form, and removing, from time to time, portions of the unconsumed fuel and the gangue in solid form from the lower portion of the de-oxidizing chamber.
2. The process of recovering metals having a low volatilizing point, which consists in highly heating, in a de-oxidizing chamber, a mixture of ore and infusible spacing lumps of several times the volume of ore, and serving to practically isolate the ore-20 portions, maintaining in the chamber a down-draft limited air-supply and producing de-oxidizing gas and a volatilizing temperature sufficient to volatilize the most of the metal, but without forming a bath of the
- 25 earthy constituents of the ore, passing the de-oxidizing gases and metal vapor through a chamber in which de-oxidizing conditions are maintained and the values recovered in metallic form, removing from time to time from the lower portion of the de-oxidizing chamber the spacing-lumps and the gangue in solid form, and collecting at the bottom of the de-oxidizing chamber any metals which may be cooled in the lower portion of
- 35 the de-oxidizing chamber.
3. The process of recovering metals which have a low volatilizing point, which consists in subjecting, in a de-oxidizing chamber, a low pile of ore mixed with several times its
- 40 volume of coke or charcoal, which is mainly in large pieces and serves practically to isolate or envelop the ore-lump groups, to a down-draft limited air-supply and producing a de-oxidizing and volatilizing temperature, a
- 45 de-oxidizing atmosphere being maintained
- in the de-oxidizing chamber, passing the de-oxidizing gas and metal vapors through a condenser, removing, from time to time, portions of the unconsumed fuel, and the gangue in solid form from the lower portion 50 of the de-oxidizing chamber, and recharging the recovered fuel with a fresh ore-charge and sufficient fresh fuel to maintain the proportions again into the de-oxidizing chamber.
4. In ore-reducing apparatus adapted to the recovery of metals having a low volatilizing point, the combination of a de-oxidizing chamber adapted to contain a mixture of ore and fuel in a stack, means for introducing fresh charges into the upper end of said de-oxidizing chamber, means for supplying air thereto in limited quantity, means for discharging the unconsumed fuel and the gangue in solid form from the lower 65 portion of the de-oxidizing chamber, a condenser communicating with the de-oxidizing chamber and adapted to maintain de-oxidizing conditions, and a pump serving to draw the de-oxidizing gases through the condens- 70 ing-chamber.
5. In ore-reducing apparatus adapted to the recovery of metals of low volatilizing point, the combination of a de-oxidizing chamber adapted to maintain a charge of 75 ore and fuel in a low stack, means for charging ore and fuel into the upper portion of said chamber, means for admitting air in limited quantity to the upper portion of said chamber, a condenser communicating 80 with the intermediate portion of said chamber, means for drawing the de-oxidizing gases through said condenser, and means for discharging the unconsumed fuel and the gangue in solid form from the bottom of the 85 de-oxidizing chamber.

ALBERT G. JONES.

In presence of—  
 NELLIE B. DEARBORN,  
 DAISY C. THORSEN.